

# UNITED STATES PATENT OFFICE.

MAX PFAFFENZELLER, OF BROOKLYN, NEW YORK.

## PROCESS OF MAKING TRANSPARENT TRANSFER-PAPER.

SPECIFICATION forming part of Letters Patent No. 522,350, dated July 3, 1894.

Application filed February 24, 1894. Serial No. 501,427. (No specimens.)

*To all whom it may concern:*

Be it known that I, MAX PFAFFENZELLER, a subject of the Emperor of Germany, residing at Brooklyn, in the county of Kings and State 5 of New York, have invented certain new and useful Improvements in Processes of Making Transparent Transfer-Paper, of which the following is a specification.

This invention has reference to an im-  
10 proved process of making transparent trans-  
fer-paper to be used in the manufacture of  
wall-paper, lithographs, &c., for transferring  
designs; and the invention consists of a pro-  
cess of making transparent transfer-paper by  
15 the following steps: first, giving a sheet of  
good paper a coat of boiled linseed-oil on  
both sides, and then permitting the paper to  
dry for some time; next, carefully wiping the  
paper on one side until it is dry and giving  
20 to the other side a second coating of linseed-  
oil and permitting it to soak into the paper;  
next, imparting a coat of lard-oil to the wiped-  
off side of the paper and also a third coat of  
linseed-oil to the opposite side, after which  
25 the paper is again hung up for drying; giv-  
ing then another coat of linseed-oil on the  
same side of the paper to which the linseed-  
oil was applied before; next, applying a coat  
of lard-oil to both sides of the paper and al-  
30 lowing the paper to dry for a long period of  
time, then rubbing the paper with a soft  
piece of cloth until the surface is dry, and ap-  
plying finally a coat of varnish, whereby the  
paper is hardened and rendered not liable to  
35 crack.

In carrying out my invention, the paper se-  
lected is preferably a good quality of white-  
paper, which is first coated on both sides  
with boiled linseed-oil, after which it is rolled  
40 up and laid aside for about forty-eight hours.  
The paper is then wiped-off carefully on one  
side by means of a soft piece of cloth or other  
absorbent material until it is perfectly dry.  
The other side receives another coat of lin-  
45 seed-oil, after which the paper is hung up for  
about twenty-four hours. At the end of this  
time, the side that was wiped off receives a  
coat of lard-oil, while the other side receives  
a third coat of boiled linseed-oil, after which  
50 the paper is hung up for drying for another  
twenty-four hours. At the end of this time

the paper receives a fourth coat of boiled  
linseed-oil on the same side to which the pre-  
ceding coat was applied, and is hung up  
again for twenty-four hours. During the 55  
drying of the paper the lard-oil serves to ab-  
sorb the white specks that are formed on that  
side of the paper coated with the linseed-oil,  
so that a clear and transparent surface is ob-  
tained. The paper receives next a coat of 60  
lard-oil on both sides and is then hung up  
for about a week, after which it is cleaned off  
on both sides with a soft piece of cloth until  
it becomes perfectly dry, when it receives a  
final coat composed of a solution of white 65  
shellac, twenty-five parts, borax five parts and  
alcohol seventy parts. The solution hardens  
the surface of the transfer paper and pre-  
vents it from cracking. All of these coats  
must be applied very thin, care being taken 70  
that all surfaces of the paper be fully coated.

When the paper is used for transferring,  
the design is traced by means of a stylus on  
the side which has received several coats of  
linseed-oil. The design thus traced is given 75  
a good coating of printing ink diluted with  
sweet oil. This coating is then rubbed off  
with a piece of clean cloth or other absorb-  
ent material, only the outlines of the draw-  
ing then remaining in black. In this condi- 80  
tion the transfer is laid on a flat form and  
the back of the same rubbed with a smooth  
steel instrument. This transfer can be used  
twenty to thirty times before fresh ink is ap-  
plied. When the paper is used by lithog- 85  
raphers, one coat of linseed-oil less than  
when it is used in the manufacture of wall-  
paper is used, for the reason that lithogra-  
phers require a somewhat finer and more pli-  
able paper for their comparatively small de- 90  
signs than wall-paper manufacturers, where  
larger designs are usually transferred, which  
require a somewhat stronger and stouter  
paper.

Having thus described my invention, I 95  
claim as new and desire to secure by Letters  
Patent—

1. The process herein described of making  
transparent transfer-paper, which consists in  
applying thin coatings of linseed-oil and 100  
lard-oil on both sides of the paper, drying the  
paper after each operation of coating, then,

before varnishing, rubbing the paper on both sides until very dry, and finally varnishing the paper, substantially as set forth.

2. The process herein-described of making transparent transfer-paper, which consists in imparting to both sides of the paper a coat of boiled linseed-oil, wiping off one side of the paper and imparting successively several coats of boiled linseed-oil to the other side, while giving a coat of lard-oil to the wiped-off side, drying the paper, and then giving a coat of lard-oil to both sides of the same,

then drying the paper for a long period of time, and then rubbing carefully both sides of the paper, so as to remove the surplus oil, and finally varnishing the paper, substantially as set forth.

In testimony that I claim the foregoing as my invention I have signed my name in presence of two subscribing witnesses.

MAX PFAFFENZELLER.

Witnesses:

PAUL GOEPEL,  
K. R. BRENNAN.